

# UNITED STATES PATENT OFFICE.

MIKE RADE RESANOVICH, OF WOODLAWN, PENNSYLVANIA.

## FIRE-EXTINGUISHING COMPOSITION.

1,411,301.

Specification of Letters Patent.

Patented Apr. 4, 1922.

No Drawing.

Application filed July 22, 1921. Serial No. 486,835.

To all whom it may concern:

Be it known that I, MIKE RADE RESANOVICH, a citizen of Austria, and a resident of Woodlawn, in the county of Beaver and State of Pennsylvania, have invented certain new and useful Improvements in Fire-Extinguishing Composition, of which the following is a specification.

My invention relates to fire extinguishing compositions, and the object of my invention is the production of a composition of this character which will be effective to quickly and completely extinguish fires even though the fire be the result of the combustion of highly inflammable substances, such as oils, gas or the like.

My composition consists of a mixture of sauerkraut brine, skim milk, aluminum salt, salt and acid, such as hydrochloric or sulfuric acid.

In preparing the composition I prefer to use the ingredients in about the following proportions:

|    |                  |            |
|----|------------------|------------|
| 25 | Sauerkraut brine | 35 gallons |
|    | Skim milk        | 10 gallons |
|    | Aluminum salt    | 4 pounds   |
|    | Salt             | 25 pounds  |
|    | Acid             | 3 quarts   |

30 The sauerkraut brine is expressed from

the sauerkraut. The mixture from which the brine is obtained preferably contains approximately four bushels of sauerkraut and approximately thirty-five gallons of liquid, chiefly water, to which twenty-five pounds of salt is added. If the water used in making the sauerkraut is cold it should be permitted to stand for approximately a month whereas if warm water is used, the liquid is ready to be used within one or two weeks.

The final composition consists of a uniform and complete solution which though possessing some viscosity is at the same time susceptible of being readily handled so that it may be readily applied to a fire. 45 When it is applied to the fire it completely arrests combustion and prevents the fire from again starting up and this is true even though the substance being consumed is highly inflammable oil or gas.

I claim:

1. A fire extinguishing composition composed of thirty-five gallons of sauerkraut brine, ten gallons of skim milk, four pounds of aluminum salt, twenty-five pounds of salt, 55 and three quarts of acid.

2. A fire extinguishing composition composed of sauerkraut brine, skim milk, aluminum salt, salt and acid.

MIKE RADE RESANOVICH.